

## UNITED STATES PATENT OFFICE

2,304,252

PROCESS OF INSOLUBILIZING HYDROXYL-  
CONTAINING SIZESOnslow B. Hager, Glenside, and Louis H. Bock  
and Alva L. Houk, Philadelphia, Pa., assignors  
to Röhm & Haas Company, Philadelphia, Pa.No Drawing. Application February 1, 1939,  
Serial No. 253,996

13 Claims. (Cl. 117--143)

This invention concerns an improved process for insolubilizing water-soluble or water-dispersible, high molecular weight compounds containing a multiplicity of hydroxyl groups. It particularly deals with the "fixation" of polymeric, hydroxyl-containing products, such as polyvinyl alcohol and the water-dispersible polyoses which include amylaceous and cellulosic finishing materials, by reaction of these compounds with a quaternary ammonium salt of the general formula



wherein R is an aliphatic hydrocarbon group, X is a salt-forming anion and R<sub>1</sub>, R<sub>2</sub>, and R<sub>3</sub> are hydrogen or alkyl groups or R<sub>1</sub> and R<sub>2</sub> jointly form an aromatic ring.

The high molecular weight, hydroxyl-containing substances which are water dispersible or water-soluble are useful for sizing or finishing fabric and paper; but they are readily redispersible by water. For many purposes it becomes desirable to provide a finish which is not readily removable by washing. No general method has heretofore been available for the treatment of sizing materials, although attempts have been made to fix starch. The setting of starch finishes by treating with quaternary organic compounds, built up from heterocyclic tertiary bases, such as pyridine, or from such tertiary amines as trimethylamine, triethylamine, triethanolamine, etc., presents various serious disadvantages. The quaternary salts from heterocyclic amines are not entirely stable in aqueous solutions, a property which interferes with their practical application and with the compounding of prepared sizing compositions. When these compounds are heated to cause fixation of the starch, toxic fumes are evolved. The quaternary salts formed from trimethylamine and the like are too stable for practical use and require excessive temperatures for their application. This results in injury to fabric as well as unsatisfactory finishes.

It is an object of this invention to provide a general method of rendering water-soluble or water-dispersible, hydroxyl-containing, high molecular weight, sizing materials relatively insoluble. It is an object of this invention to provide a superior means for improving the fastness of water-dispersible, sizing materials on fabric without causing deterioration of fabric or finish and without evolving toxic fumes.

We have found that, when hydroxyl-containing, sizing materials are heated with a quaternary compound of the general formula given above, they become insolubilized. If fabric, yarn, or fibers are treated with such a sizing material and with the said quaternary compound, and the sized fabric, yarn or fibers are then heated, the sizing and quaternary compound react and the sizing becomes "fixed" and fast to ordinary washing. Fabric sized by this method is permanently stiffened.

Application of size and of fixing agent is preferably performed in a single bath, but treatments with these substances in separate baths are also effective. Mildly acidic catalysts or alkaline catalysts seem to assist in the reaction between the sizing materials and the fixing agent, but are not essential. For example, it is helpful to add ammonium chloride, sodium acetate, borax, sodium bicarbonate, sodium carbonate, and the like. After application of the sizing materials and the fixing agent to fabric, yarn, or fiber, the treated material may be dried in a separate operation before the final heating, but such drying is not essential as it may be performed as part of the heating procedure in which the size and agent are reacted. It is sometimes desirable to wash the sized fabric before the last finishing operation in order to remove salts, decomposition products, or excess, unfixed sizing material.

Quaternary ammonium compounds of the above general type possess advantages over other quaternary compounds in having such a degree of stability that they may be incorporated in sizing preparations, whether in dry form or in paste form, yet they react under such conditions of moisture, temperature, and pH that fibers or fabrics are not unduly tendered. No noxious or toxic fumes are evolved. By proper choice of the individual compound different degrees of stiffness and qualities of finish may be produced. These compounds are useful with any of the sizing materials which contain a multiplicity of hydroxyl groups.

Quaternary ammonium salts of the type found particularly effective may be prepared by reacting a tertiary amine carrying a  $\beta,\gamma$ -unsaturated hydrocarbon group, such as allyl dimethylamine or benzyl dimethylamine, with a halo-methyl ether, such as caproxyethyl chloride or butyloxyethyl bromide. Certain suitable quaternary salts may also be prepared by steps involving (1) the synthesis of an alkoxyethyl tertiary amine, such as lauryloxyethyl dimethyl amine, which is obtained by reacting a primary

alcohol, formaldehyde, and a secondary amine, and (2) the reaction of the alkoxyethyl tertiary amine with a suitable unsaturated agent for alkylation, such as methallyl bromide, allyl chloride, benzyl chloride, or the like.

The compounds which are most readily available may be conveniently grouped in the following general formula



wherein R' is a member of the class consisting of allyl,  $\beta$ -methallyl, crotyl and benzyl groups. The group R in the above formulae may be any aliphatic hydrocarbon radical. It may possess a straight chain or a branched chain; it may be saturated or unsaturated. We have observed that the maximum degree of fixation of starch occurs when the carbon atom content of R is about four to eight, but fewer carbon atoms or more carbon atoms in R still yield useful compounds. Shorter groups tend to give somewhat crisper finishes, while longer groups give softer finishes, and if sufficiently long (as C<sub>14</sub> or more), some-what water-resistant effects.

Typical compounds which give the desired resistance of sizes and finishes to water and washing include



The water-soluble or water-dispersible, poly-hydroxy, high molecular weight compounds which are useful for sizing or finishing include cellulose ethers, such as the water-soluble forms of methyl and ethyl cellulose, hydroxyethyl cellulose and the like, polyvinyl alcohol, and the starches and starchy products, including corn, rice, tapioca, sago, wheat, and potato starch, flours containing starches, modified and treated starches, converted starches, etc. Other materials which are commonly applied with starch, such as fillers, pigments, softeners, resins, etc., may also be incorporated in the finishing mixtures.

The polyhydroxy sizing materials react at slightly elevated temperatures with the quaternary salts described above to form insoluble complexes which thus provide improved finishes. In carrying out sizing operations with fabric about two parts of the quaternary ammonium compound may be added to one to ten parts of a water-dispersible size in a treating bath. The sizing preparation is used to impregnate or coat fabric by any suitable means, such as padding. Then, the fabric, with or without drying, is heated to a temperature sufficiently high to bring

about reaction of the sizing material and the quaternary ammonium compound.

While a one-bath process is usually to be desired, the equivalent result is obtained from a two-bath process in which size is applied from one bath and the quaternary ammonium compound from a second bath. As yet another procedure, a size may be partially reacted with one of the quaternary ammonium compounds of the type described above by heating the size with the quaternary compound. The partially reacted size is then applied to fibers or fabric and completely insolubilized thereon by a final heating of the sized fibers or fabric.

15 The temperature required to set the size is over 100° C. In general a temperature of 120° to 140° C. for fifteen minutes or more will render size permanently insoluble. In plant operations the heating step is accomplished on hot cans or in closed tenters, loop driers and the like.

20 To illustrate the general process the following specific examples are given:

#### Example 1

25 Cotton yarn was treated with a preparation containing 2 parts of a 26% solution of cetyloxy-methyl dimethyl benzyl ammonium chloride and 40 parts of a 4% aqueous solution of ethyl cellulose. The excess was squeezed off and the yarn dried at room temperature. It was then heated in the oven at 125° C. for one-half hour. A stiff coating resulted, which softened when wet but regained its stiffness when dried. It was not removed by washing.

#### Example 2

30 Cotton lawn was coated with an aqueous solution containing 1.2% of capryloxyethyl dimethyl benzyl ammonium chloride, 0.25% of sodium bicarbonate, and 4% of water-soluble ethyl cellulose. The excess was squeezed off and the cloth dried at room temperature. It was heated at 125° C. for one-half hour, washed twice, and ironed. A stiff, full finish was obtained which was not removed by laundering.

#### Example 3

35 Cotton sheeting was coated with an aqueous solution containing 2.7% of methyl cellulose, 0.5% sodium acetate, and 8% of capryloxyethyl dimethyl benzyl ammonium chloride. It was squeezed, air-dried, and heated at 125° C. for one-half hour. A moderately stiff fabric resulted. After the sized fabric was washed and dried, it showed a weight increase of 6.03%.

#### Example 4

40 Cotton lawn was coated with an aqueous solution containing 2.4% lauryloxyethyl dimethyl methallyl ammonium chloride and 4.5% hydroxyethyl cellulose. It was squeezed and air-dried, then heated at 125° C. for one-half hour. The material was very stiff even after washing.

#### Example 5

45 Woolen cloth was coated with an aqueous solution containing 4.5% of isobutyloxyethyl dimethyl benzyl ammonium chloride and 3.3% of water-soluble ethyl cellulose. The excess was pressed off and the cloth air-dried, then heated at 125° C. for one-half hour. The material was very stiff, retaining the stiffness after washing.

#### Example 6

50 A pure silk fabric was coated with an aqueous solution containing 2.25% of capryloxyethyl di-

methyl benzyl ammonium chloride, 0.5% of disodium phosphate, and 7.25% of potato starch. The excess was squeezed off and the cloth dried at room temperature. It was heated at 120° C. for one-half hour and washed. A stiff finish resulted, permanent to washing.

*Example 7*

A viscose rayon fabric was coated with an aqueous solution containing 6.2% ethoxymethyl dimethyl benzyl ammonium chloride and 3.0% of water-soluble ethyl cellulose. It was squeezed, dried, and heated one-half hour at 125° C. Good stiffening resulted, retained after washing and drying.

*Example 8*

Cotton sheeting was coated with a solution containing 4.3% of methoxymethyl dimethyl benzyl ammonium chloride and 3.3% of water-soluble ethyl cellulose. The excess was squeezed off, the cloth dried and heated at 125° C. for one-half hour. It was given two washes, retaining good stiffness.

*Example 9*

Cotton sheeting was coated with an aqueous solution containing 3.7% of water-soluble ethyl cellulose and 2.7% of a compound obtained by the reaction of benzyl dimethylamine with a chloromethyl ether of an alcohol having an iodine number of 44 and a hydroxyl number of 228. The cloth was squeezed, dried, and heated one-half hour at 125° C. It gave a very stiff finish, permanent to washing, and exhibited some water-repellency.

*Example 10*

Cotton lawn was coated with a solution of 1 part of 26% cetyl oxymethyl dimethyl benzyl ammonium chloride in 3 parts of 4% water-soluble ethyl cellulose. It was squeezed, dried, and heated at 120° C. for one-half hour. After washing, it was fairly stiff and very repellent to water. It had gained in weight 21%.

*Example 11*

Cotton sheeting was coated with an aqueous solution of 3.7% tapioca starch and 6.5% cetyl oxymethyl dimethyl benzyl ammonium chloride. The excess was squeezed out, the cloth dried, and heated one-half hour at 125° C. The cloth was fuller, with slight stiffening, and was water-repellent.

*Example 12*

A coating composition comprising 11.3% of polyvinyl alcohol and 6.5% capryloxymethyl dimethyl benzyl ammonium chloride was adjusted to a pH of 5.8 with acetic acid, and applied to cotton sheeting, dried and heated one-half hour at 130° C. and washed. The cloth retained a stiff finish resistant to further washing.

*Example 13*

A 68 x 72, unfinished mercerized nainsook was impregnated on a quetch with a solution containing 3% hydroxyethyl cellulose and 8% caproxy-methyl dimethyl benzyl ammonium chloride. The cloth was dried on a frame at 220-230° F. It was then dampened and passed through a hydraulic calender and a friction calender maintained at 280° F. A final cure for ten minutes at 290° F. in a loop drier was given the cloth. The cloth was highly glazed, firm, yet soft and flexible, of good draping qualities. The firmness was retained on washing.

*Example 14*

An unmercerized, vat blue, 80 x 80, 4-*yd.* percale was padded with moderate pressure through a solution containing 1.5% hydroxyethyl cellulose and 4% caproxy-methyl dimethyl benzyl ammonium chloride. The cloth was dried at 37° in a closed tenter at 220-230° F. From the frame the fabric was baked for ten minutes at 290° F. in a loop drier with good circulation of air and calendered. The fabric was made full-bodied and given a slight degree of firmness and a well-filled appearance. These properties were retained on laundering.

This process of improving the fastness of water-dispersible sizes may be applied to yarn, fabric, thread or fibers of any material, which may be heated over 100° C. without impairing the properties of the sized material. It may thus be applied to cotton, linen, paper, straw, jute, hemp, the various synthetic fibers, etc.

We claim:

1. A method for improving the wash-fastness on textile material of hydroxyl-containing size selected from the group consisting of water-soluble cellulose ethers, polyvinyl alcohol and starch sizes, which comprises treating the textile material with said size and a quaternary ammonium salt of the formula—



wherein R represents an aliphatic hydrocarbon group, R' represents a group selected from allyl,  $\beta$ -methallyl, crotyl, and benzyl radicals, and X represents a salt-forming anion, and subsequently heating the treated material to effect reaction between the size and the quaternary ammonium salt.

2. A method for improving the wash-fastness on textile material of a starch size, which comprises treating the textile material with said size and a quaternary ammonium salt of the formula—



50 wherein R represents an aliphatic hydrocarbon group, R' represents a group selected from allyl,  $\beta$ -methallyl, crotyl, and benzyl radicals, and X represents a salt-forming anion, and subsequently heating the treated material to effect reaction between the size and the quaternary ammonium salt.

55 3. A method for improving the wash-fastness on textile material of polyvinyl alcohol, which comprises treating the textile material with said alcohol and a quaternary ammonium salt of the formula—



60 wherein R represents an aliphatic hydrocarbon group, R' represents a group selected from allyl,  $\beta$ -methallyl, crotyl, and benzyl radicals, and X represents a salt-forming anion, and subsequently heating the treated material to effect reaction between said alcohol and the quaternary ammonium salt.

65 4. A method for improving the wash-fastness on textile material of a water-soluble cellulose ether, which comprises treating the textile mate-

rial with said ether and a quaternary ammonium salt of the formula—



wherein R represents an aliphatic hydrocarbon group, R' represents a group selected from allyl,  $\beta$ -methallyl, crotyl, and benzyl radicals, and X represents a salt-forming anion, and subsequently heating the treated material to effect reaction between said ether and said salt.

5. A method for improving the wash-fastness on textile material of hydroxyl-containing size selected from the group consisting of water-soluble cellulose ethers, polyvinyl alcohol and starch sizes, which comprises treating the textile material with said size and a quaternary ammonium salt of the formula—



wherein R represents an aliphatic hydrocarbon group and X represents a halogen, and subsequently heating the treated material to effect reaction between the size and the quaternary ammonium salt.

6. A method for improving the wash-fastness on textile material of a starch size, which comprises treating the textile material with said size and a quaternary ammonium salt of the formula—



wherein R represents an aliphatic hydrocarbon group and X represents a halogen, and subsequently heating the treated material to effect reaction between the size and the quaternary ammonium salt.

7. A method for improving the wash-fastness on textile material of polyvinyl alcohol, which comprises treating the textile material with said alcohol and a quaternary ammonium salt of the formula—



wherein R represents an aliphatic hydrocarbon group and X represents a halogen, and subsequently heating the treated material to effect reaction between the size and the quaternary ammonium salt. 55

8. A method for improving the wash-fastness on textile material of a water-soluble cellulose ether, which comprises treating the textile material with said ether and a quaternary ammonium salt of the formula—



10 wherein R represents an aliphatic hydrocarbon group and X represents a halogen, and subsequently heating the treated material to effect reaction between the size and the quaternary ammonium salt.

15 9. A method for improving the wash-fastness on textile material of hydroxyl-containing size selected from the group consisting of water-soluble cellulose ethers, polyvinyl alcohol and starch sizes, which comprises treating the textile material with said size and caproxyethyl dimethyl benzyl ammonium chloride, and subsequently heating the treated material to effect reaction between the size and caproxyethyl dimethyl benzyl ammonium chloride.

20 10. A method for improving the wash-fastness on textile material of starch size which comprises treating the textile material with said size and caproxyethyl dimethyl benzyl ammonium chloride, and subsequently heating the treated material to effect reaction between the size and caproxyethyl dimethyl benzyl ammonium chloride.

25 11. A method for improving the wash-fastness on textile material of hydroxyl-containing size from the group consisting of water-soluble cellulose ethers, polyvinyl alcohol and starch sizes, which comprises treating the textile material with said size and cetoxyethyl dimethyl benzyl ammonium chloride, and subsequently heating the treated material to effect reaction between the size and cetoxyethyl dimethyl benzyl ammonium chloride.

30 12. A method for improving the wash-fastness on textile material of a water-soluble cellulose ether size which comprises treating the textile material with said size and cetoxyethyl dimethyl benzyl ammonium chloride, and subsequently heating the treated material to effect reaction between the size and cetoxyethyl dimethyl benzyl ammonium chloride.

35 13. The method of claim 12 in which the cellulose ether is a water-soluble ethyl cellulose.

ONSLOW B. HAGER.  
LOUIS H. BOCK.  
ALVA L. HOUK.